

# UNITED STATES PATENT OFFICE.

WILLIAM O. BRADSTREET, OF GRATIS, OHIO.

## IMPROVEMENT IN PAINT-RESTORING COMPOUNDS.

Specification forming part of Letters Patent No. 133,195, dated November 19, 1872.

*To all whom it may concern:*

Be it known that I, WILLIAM O. BRADSTREET, of Gratis, in the county of Preble and State of Ohio, have invented a new and valuable Improvement in Chemical Compounds, to be known as "Paint-Restorer;" and I do hereby declare that the following is a full, clear, and exact description of the same.

This invention has relation to a new chemical compound, to be known as a "paint-restorer;" and it consists in the combination of the following-named ingredients, substantially as hereinafter described.

Take five gallons of linseed-oil, boil it slowly for thirty minutes; then remove from the fire, and while hot add slowly one ounce of sugar of lead, one ounce of sulphate of zinc, and one ounce of red lead; stir the mixture well, and it is ready for use.

The purpose of this compound is to restore the color and gloss of paint. It is to be applied to any color with a clean brush, and, when properly made and laid on, will preserve the freshness of the color for several years.

What I claim as my invention, and desire to secure by Letters Patent, is—

The combination of the ingredients herein stated, substantially as and for the purpose set forth.

In testimony that I claim the above I have hereunto subscribed my name in the presence of two witnesses.

WILLIAM O. BRADSTREET.

Witnesses:

J. M. BRADSTREET,  
JOHN SMALLEY.